# EUROPEAN PATENT SPECIFICATION

(11) **EP 3 467 138 B1**
(45) Date of publication and mention of the grant of the patent: **24.11.2021**
(21) Application number: 17194723.7
(22) Date of filing: 04.10.2017
(51) Int. Cl.: C22F 1/04

(54) **METHOD FOR FORMING ALUMINUM ALLOY BLANK**
VERFAHREN ZUR HERSTELLUNG EINES ALUMINIUMLEGIERUNGSROHLINGS
PROCÉDÉ DE FORMATION D'ÉBAUCHE D'ALLIAGE D'ALUMINIUM

(43) Date of publication of application: 10.04.2019
(73) Proprietor: Automation, Press and Tooling, A.P. & T AB, 514 32 Tranemo (SE)
(72) Inventor: Koroschetz, Christian, 438 38 Landvetter (SE); Anyasodor, Gerald, 523 34 Ulricehamn (SE)
(74) Representative: AWA Sweden AB

(56) References cited:
- EP-A2- 2 987 878
- WO-A1-2010/032002
- WO-A1-2017/021742
- WO-A1-2017/093767
- DE-A1-102012 007 213

## Description

### Technical Field

The present disclosure relates to a heat treatment method of blank sheets of aluminum alloys, and especially to a method suitable for blank sheets of any aluminum alloy grade, composition or temper.

### Background

In especially the automotive industry, the hot forming of blank sheets is important, in particular hot forming of blank sheets of high strength aluminum alloys. There are numerous methods known for forming aluminum alloy blanks. E.g. the hot forming die quenching methods as presented in WO2010/032002 and WO2015/136299.

However, such known methods have several drawbacks. For instance, these methods are not suitable for all aluminum alloy grades. The method in WO2010/032002 may be suitable for AA6082 material, but not for any AA7xxx material. Further, the aluminum alloy grade material compositions and tempers may vary from different material suppliers. The resulting formed components using the known methods are very sensitive to different compositions and tempers.

Further, the known processes have problems in being suitable for mass production due to lack of stability, repeatability and accuracy of the formed components.

EP2987878 A2 discloses a method of forming an AI alloy blank comprising steps of heating the blank for solution heat treatment, shielding a part of the blank such that a first part of the blank is quenched to a temperature between 150-200°C and a second part of the blank is quenched to below 150°C, forming the blank during or after the quenching, and ageing the formed blank. DE102012007213 A1 discloses a method comprising heating aluminum sheet to solution annealing temperature and molding and simultaneously quenching. Consequently, there is a need for production method for forming aluminum alloy blank sheets which alleviate the mentioned drawbacks of known technology.

### Summary

It is an object of the present invention to provide an improved solution that alleviates the mentioned drawbacks with present devices. Furthermore, it is an object to provide a method resulting in improved accuracy of the formed parts.

The invention is defined by the appended independent claim 1, with embodiments being set forth in the appended dependent claims 2-4.

By using a method according to the present invention, a method is provided that, with high accuracy of the formed components and low amount of springbacks, is suitable for AA6082 or 7xxx series aluminum alloy grade sheet blank.

The time in which the blank is kept at or above the solution heat treatment (SHT) temperature may be chosen to be sufficient to ensure maximum concentration of hardening elements, such as copper, zinc, magnesium, manganese, silicon etc. in the solid solution. The concentration and rate of dissolution of these elements in the solid solution may increase with increasing temperature.

By cooling the blank at a specific cooling rate the SHT composition of the solid solution may be preserved at the intermediate temperature. If the blank were to be cooled in a too slow rate, the alloying elements may diffuse through the solid solution and concentrate at the grain boundaries, in large voids, undissolved particles or other undesired locations. To achieve improved strength properties of the formed part, it may be desirable to avoid such recrystallization and decrease the diffusion process and maintain the alloying elements in the solid solution by providing a rapid cooling. The cooling rate to achieve this may be selected depending on the aluminum alloy grade and composition of the blank. Further, a quenching rate may be selected depending on the aluminum alloy grade and composition of the blank.

In one embodiment, the forming tool may be preheated to the intermediate temperature. The blank may thereby be formed at the intermediate temperature. The temperature of the blank may thereby be controlled during the forming, which may improve the accuracy in the properties of the final formed component.

In one embodiment, the blank may be kept at the intermediate temperature during the forming step in the forming tool. The temperature of the tool may be controlled in order to keep the temperature of both the tool and the blank stable at the intermediate temperature during the forming. After the forming, the temperature of the forming tool may be controlled in order to quench the formed blank to room temperature. A temperature control function may be provided for the forming tool in order to control the temperature of the forming tool to the intermediate temperature throughout the forming step.

In one embodiment, the forming and the quenching may be performed in separate forming tools. A first forming tool may form the blank at the intermediate temperature, and a second forming tool may quench the blank to room temperature. In a further embodiment, the first forming tool may be preheated to the intermediate temperature, thereby keeping the blank at the intermediate temperature during the forming. The blank may then be transferred to the second forming tool, quenching the blank to room temperature. The second forming tool may be a cold forming tool. Alternatively, the first forming tool may not be preheated, thereby cooling the blank during the forming. The blank may then in the second forming tool be quenched in a controlled manner to room temperature in the second forming tool.

### Brief Description of the Drawings

The invention will in the following be described in more detail with reference to the enclosed drawings, wherein:
Fig. 1 shows a flow chart of a method according to an embodiment of the invention;
Fig. 2 shows a block scheme of a system according to an embodiment of the invention;
Fig. 3 shows a diagram view of a process of the method according to an embodiment of the invention;
Fig. 4 shows a flow chart of a method according to an embodiment of the invention;
Fig. 5 shows a block scheme of a system according to an embodiment of the invention; and
Fig. 6 shows a diagram view of a process of the method according to an embodiment of the invention.

### Description of Embodiments

The present invention will be described more fully hereinafter with reference to the accompanying drawings, in which preferred embodiments of the invention are shown. This invention may, however, be embodied in many different forms and should not be construed as limited to the embodiments set forth herein; rather, these embodiments are provided so that this disclosure will be thorough and complete, and will fully convey the invention to those skilled in the art. In the drawings, like numbers refer to like elements.

As illustrated in figure 1, a method 100 according to an embodiment of the present invention comprises a first step of heating 102 a 6xxx or 7xxx series Al alloy blank 2 to the solutionization (SHT) temperature for the specific alloy of the blank 2. As further seen in fig. 2, a blank forming system 1 is provided, wherein the heating 102 is performed in a heating station 10. In the heating station 10, when the blank 2 has reached its SHT temperature or above, the temperature of the blank 2 is kept at the SHT temperature or above until the solutionization of the alloy of the blank 2 is complete.

In a next step, the blank 2 is cooled 104 to an intermediate temperature. In the blank forming system 1, the cooling 104 is performed at a cooling station 20. The intermediate temperature is selected for the alloy of the blank 2 at which temperature the kinetic movement for the alloy stops. The cooling 104 is performed at a cooling rate high enough such that recrystallization in the alloy of the blank 2 does not occur.

In a next step, the blank 2 is formed 106 in a forming tool 32 at a press station 30 in the blank forming system 1. The press station 30 may be a press suitable for aluminum alloy blank sheet forming, such as a hydraulic press, a servo press (servo hydraulic or servo mechanical).

After forming 106 of the blank 2, the formed blank 2', or formed component 2', is quenched 108 in the forming tool 32 to room temperature.

Finally, the formed blank 2' is artificially aged 110 at an ageing station 40. The ageing process is provided to control and limit the recrystallization in the alloy material of the blank 2.

Fig. 3 illustrates the blank forming method 100 according to an embodiment of the present invention. The blank 2 is heated from room temperature T_{E} to the SHT temperature T_{SHT}, and kept at the T_{SHT} for a necessary time t₁-t₂ as discussed above. At t₂ the blank 2 is rapidly cooled to the intermediate temperature T_{ITM} at the necessary cooling rate as discussed above. The blank 2 is then formed during t₂-t₃ in the forming tool 32. At t₃ the formed blank 2' is quenched to room temperature T_{E}.

At the ageing station 40, the formed component 2' is processed for artificial ageing by being heated to an ageing temperature T_{A}. The component 2' is kept at the ageing temperature T_{A} during a period t₅-t₆ until the ageing process is complete. The time t₃-t₄ provides a transfer of the formed blank to the ageing station 40.

The blank 2 is transferred between the different stations 10, 20, 30, 40. The transfer may be performed such that minimal heat loss in the blank 2 is achieved.

Figs. 4 and 5 illustrates a method 200 and system 3 according to an embodiment of the invention. The steps of heating 202 and cooling 204 correspond to the steps 102 and 104 as discussed above. Next, the blank 2 is formed 206 in a preheated first forming tool 32a at a press station 30 in the blank forming system 3. The first forming tool 32a is preheated to the intermediate temperature. The blank 2 is thereby not further cooled when arranged in the first forming tool 32a. The intermediate temperature may be kept in the first forming tool 32a and the blank 2 throughout the forming process 106.

Next, the formed blank is moved to a separate cold second forming tool 32b. In the cold second forming tool 32b, the blank is quenched to room temperature. The cold second forming tool 32b may further form and quench the blank to its final shaped component.

Fig. 5 further illustrates an optional arrangement of ageing which can be used for either of the above presented embodiments. In such ageing embodiment, a first pre-ageing step is performed at a pre-ageing station 40a, in which the formed component 2' is heated to the ageing temperature T_{A}, kept at T_{A} until the pre-ageing is complete and then cooled to room temperature T_{E}. After transfer to a second ageing station 40b, the component 2' is again heated to T_{A}, kept at T_{A} for a time period and thereafter cooled to room temperature T_{E}, to provide a paint baking of the component 2'. Alternatively, the component can be heated to a different temperature in the paint baking process than the temperature T_{A} in the pre-ageing process. A two-step ageing process is thereby provided comprising pre-ageing and paint baking.

Preferably, the pre-ageing process is integrated in the forming/stamping line, and performed in direct connection to the forming of the component 2'. The paint baking process may be performed at a later stage, whichever may be suitable for the production line.

The use of the pre-ageing process prevents natural ageing after stamping in the second forming tool. Otherwise, natural ageing may occur after about 30 minutes for 7xxx series Al alloy materials or about one hour for 6xxx series Al alloy materials. The paint baking process cannot take effect on the formed component to achieve peak hardness. The pre-ageing process further enables post processing activities such as transport to another location, storage for a required period before assembly or joining operations. Then, the paint baking operation may be performed at the most suitable time to provide optimal peak hardness in a short cycle time and at a low cost. This may e.g. be after joining the formed component 2' to a desired assembly.

Fig. 6 illustrates the process blank forming method 200 according to an embodiment of the present invention. The blank 2 is heated from room temperature T_{E} to the SHT temperature T_{SHT}, and kept at the T_{SHT} for a necessary time t₁-t₂ as discussed above. Between t₂ and t₃, the blank 2 is cooled to the intermediate temperature T_{ITM} at the necessary cooling rate as discussed above. The blank 2 is then formed during t₃-t₄ in the preheated first forming tool 32a. Between t₄ and t₅ the formed blank 2' is quenched to room temperature T_{E} in the second forming tool 32b.

Fig. 6 further illustrate the process of the embodiment comprising a pre-ageing and a paint baking step as discussed above. At the pre-ageing station 40a, the formed blank 2' is processed for artificial ageing by being heated to the ageing temperature T_{A} and kept at the ageing temperature T_{A} during a period t₇-t₈. After being cooled to room temperature, the blank 2' is in the second ageing station 40b again heated to the ageing temperature T_{A} and kept at T_{A} between t₁₁-t₁₂ until the ageing process is complete. The blank 2' formed to a final shaped component is then again cooled to room temperature T_{E}.

In the drawings and specification, there have been disclosed preferred embodiments and examples of the invention and, although specific terms are employed, they are used in a generic and descriptive sense only and not for the purpose of limitation, the scope of the invention being set forth in the following claims.

## Claims

1. A method (100) of forming a AA6082 alloy blank or a 7xxx series alloy blank (2), wherein the method comprises the steps of:
heating (102) the blank to a solutionization (SHT) temperature (T_{SHT}) for the alloy of the blank at a heating station (10) and keeping the blank at said SHT temperature until SHT is complete,
cooling (104) the blank at a cooling station (20) to an intermediate temperature (T_{ITM}) and at a cooling rate that is high enough such that recrystallization in the alloy of the blank does not occur, wherein for a AA6082 alloy blank the intermediate temperature is between 300-350ºC and the cooling rate is at least 30 K/s, and for a 7xxx series alloy blank the intermediate temperature is between 400-420ºC and the cooling rate is at least 50 K/s,
forming (106) the blank in a forming tool (32),
quenching (108) the formed blank (2') to room temperature (T_{E}),
pre-ageing the formed and quenched blank in a pre-ageing station (40a) within one hour of the quenching of the formed blank for a AA6082 alloy blank and within 30 minutes of the quenching of the formed blank for a 7xxx series alloy blank, in which pre-ageing the formed and quenched blank is heated to an ageing temperature (T_{A}), kept at the ageing temperature during a time period, and cooled to room temperature.

2. The method according to any of the preceding claims, wherein the forming tool (32) is preheated to the intermediate temperature (T_{ITM}).

3. The method according to any of the preceding claims, wherein the blank (2) is kept at the intermediate temperature (T_{ITM}) during the forming (106) in the forming tool (32).

4. The method according to any of the preceding claims, wherein the forming is performed in a first forming tool (32a) and the quenching is performed in a second forming tool (32b).

## Patentansprüche

1. Verfahren (100) zum Bilden eines AA6082 Al-Legierungsrohlings oder eines Al-Legierungsrohlings der Serie 7xxx (2), das Verfahren umfassend die Schritte:
Erhitzen (102) des Rohlings auf eine Lösungstemperatur (SHT-Temperatur) (T_{SHT}) für die Legierung des Rohlings an einer Heizstation (10) und Halten des Rohlings auf dieser SHT-Temperatur bis die SHT abgeschlossen ist,
Abkühlen (104) des Rohlings an einer Kühlstation (20) auf eine Zwischentemperatur (T_{ITM}) und mit einer Kühlgeschwindigkeit, welche hoch genug ist, dass keine Umkristallisation in der Legierung des Rohlings erfolgt, wobei für einen AA6082-Al-Legierungsrohling die Zwischentemperatur 300 - 350 °C und die Kühlgeschwindigkeit mindestens 30 K/s beträgt, und für einen Al-Legierungsrohling der Serie 7xxx die Zwischentemperatur 400 - 420 °C und die Kühlgeschwindigkeit mindestens 50 K/s beträgt,
Formen (106) des Rohlings in einem Formwerkzeug (32),
Abschrecken (108) des geformten Rohlings (2') auf Raumtemperatur (T_{E}),
Voraltern des geformten und abgeschreckten Rohlings in einer Voralterungsstation (40a) innerhalb einer Stunde nach dem Abschrecken des geformten Rohlings für einen AA6082-Al-Legierungsrohling und innerhalb von 30 Minuten nach dem Abschrecken des geformten Rohlings für einen Legierungsrohling der Serie 7xxx, wobei das Voraltern des geformten und abgeschreckten Rohlings das Erhitzen auf eine Alterungstemperatur (T_{A}), das Halten auf der Alterungstemperatur für einen bestimmten Zeitraum und das Abkühlen auf Raumtemperatur umfasst.

2. Verfahren nach einem der vorstehenden Ansprüche, wobei das Formwerkzeug (32) auf die Zwischentemperatur (T_{ITM}) vorgeheizt wird.

3. Verfahren nach einem der vorstehenden Ansprüche, wobei der Rohling (2) während des Formens (106) im Formwerkzeug (32) auf der Zwischentemperatur (T_{ITM}) gehalten wird.

4. Verfahren nach einem der vorstehenden Ansprüche, wobei das Formen in einem ersten Formwerkzeug (32a) vorgenommen wird, und das Abschrecken in einem zweiten Formwerkzeug (32b) vorgenommen wird.

## Revendications

1. Procédé (100) de formation d'une ébauche d'alliage pour une ébauche d'alliage d'AI AA6082 ou une ébauche d'alliage d'AL de la série 7xxx (2), dans lequel le procédé comprend les étapes consistant à :
chauffer (102) l'ébauche à une température (T_{SHT}) de mise en solution (SHT) pour l'alliage de l'ébauche au niveau d'une station de chauffage (10) et maintenir l'ébauche à ladite température SHT jusqu'à ce que la SHT soit terminée,
refroidir (104) l'ébauche au niveau d'une station de refroidissement (20) à une température intermédiaire (T_{ITM}) et à une vitesse de refroidissement qui est suffisamment élevée pour que la recristallisation dans l'alliage de l'ébauche ne se produise pas, dans lequel pour une ébauche d'alliage d'AI AA6082, la température intermédiaire est comprise entre 300 et 350 °C et la vitesse de refroidissement est d'au moins 30 K/s, et pour une ébauche d'alliage d'AL de la série 7xxx, la température intermédiaire est comprise entre 400 et 420 °C et la vitesse de refroidissement est d'au moins 50 K/s,
former (106) l'ébauche dans un outil de formage (32),
tremper (108) l'ébauche formée (2') à température ambiante (T_{E}),
pré-vieillir l'ébauche formée et trempée dans une station de pré-vieillissement (40a) dans l'heure qui suit la trempe de l'ébauche formée pour une ébauche d'alliage d'AI AA6082 et dans les 30 minutes qui suivent la trempe de l'ébauche formée pour une ébauche d'alliage d'AL de la série 7xxx, dans ledit pré-vieillissement, l'ébauche formée et trempée est chauffée à une température de vieillissement (T_{A}), maintenue à la température de vieillissement pendant une certaine période de temps, et refroidie à température ambiante.

2. Procédé selon l'une quelconque des revendications précédentes, dans lequel l'outil de formage (32) est préchauffé à la température intermédiaire (T_{ITM}).

3. Procédé selon l'une quelconque des revendications précédentes, dans lequel l'ébauche (2) est maintenue à la température intermédiaire (T_{ITM}) pendant le formage (106) dans l'outil de formage (32).

4. Procédé selon l'une quelconque des revendications précédentes, dans lequel le formage est réalisé dans un premier outil de formage (32a) et la trempe est réalisée dans un second outil de formage (32b).
